

## UNITED STATES PATENT OFFICE

1,921,416

## ALLOY

Robert H. Leach, Fairfield, Conn., assignor to  
Handy & Harman, New York, N. Y., a Corpora-  
tion of New York

No Drawing. Application May 4, 1933  
Serial No. 669,370

## 4 Claims. (Cl. 75—1)

This invention relates to alloys used for brazing and welding and is concerned more particularly with a novel quaternary alloy which has relatively low melting and flow points and which can be used with great facility in producing joints 5 of high tensile strength.

The new alloy includes silver varying from 4% to 36%, copper varying from 55% to 80%, tin varying from 5% to 15%, and phosphorus varying from 2% to 6%, the range limits given being 10 approximate. Specific examples of the new alloys may have approximate compositions as follows:

|    |             | Per cent |
|----|-------------|----------|
| 15 | 1. Silver   | 4.0      |
|    | Copper      | 78.1     |
|    | Tin         | 13.4     |
|    | Phosphorous | 4.5      |
| 20 | 2. Silver   | 14.3     |
|    | Copper      | 69.5     |
|    | Tin         | 11.2     |
|    | Phosphorus  | 5.0      |
| 25 | 3. Silver   | 14.4     |
|    | Copper      | 70.4     |
|    | Tin         | 11.4     |
|    | Phosphorus  | 3.8      |
| 30 | 4. Silver   | 24.0     |
|    | Copper      | 63.3     |
|    | Tin         | 9.5      |
|    | Phosphorus  | 3.2      |
| 35 | 5. Silver   | 36.0     |
|    | Copper      | 54.5     |
|    | Tin         | 7.1      |
|    | Phosphorus  | 2.4      |

These and other alloys within the ranges mentioned offer the advantage of having melting 40 points which are substantially lower than those of the alloys commonly known as "silver solder", they are cheaper than silver solders, and because of the presence of the phosphorus, they may be employed with little or no flux.

45 The new alloys may be said to represent combinations of the silver-copper eutectic and the copper-tin-phosphorus eutectic in proportions ranging from 1 to 1 of each eutectic to 1 of the silver-copper eutectic to 18 of the copper-tin- 50 phosphorus eutectic with such small variations as may be desirable to obtain the best combination of thermal and physical properties. The silver-copper eutectic contains approximately 72% silver and 28% copper, while the copper-tin-phosphorus eutectic contains approximately 55

81% copper, 14.2% tin, and 4.8% phosphorus. Accordingly, in developing this new alloy, I have departed in some instances from this combination of the eutectics by varying the amounts of the ingredients. For example, in an alloy containing, silver 10%, copper 73.5%, tin 12.2%, and phosphorus 4.1%, which represents a combination of eutectics, it is possible to increase the copper to 75.7% and lower the phosphorus to 2.1%, the tin and silver remaining the same, without changing the characteristics of the alloy so that it cannot be used for brazing purposes. 60

The alloys within the ranges specified have closely similar melting and flow points as, for example, the alloy given in example No. 1 above 70 and containing 4% of silver has a melting point of 1130° F. and a flow point of 1230° F. whereas the alloy given in example No. 5 which contains 36% silver has a melting point of 1115° F. and a flow point of 1295° F. It will thus be apparent that the thermal properties can be kept within reasonably close limits over a considerable range of composition and allow the use of an alloy with low silver content for brazing or welding purposes in those cases where the better physical properties of the alloys with higher silver content are not necessary. 80

Substantially all the alloys having the compositions within the ranges mentioned can be hot-rolled at 900° F. to 1000° F., and the ease with 85 which they can be rolled increases with the silver content. When used as a solder and without a flux, the alloys flow along the seam or through the joint to a substantial extent, and tensile strength tests of copper butt joints made with the 90 solders show average strengths in pounds per square inch ranging from 19,000 to 29,100. The butt joints thus made can be bent to an angle of 180° and hammered flat without cracking.

By reason of the relatively low temperatures at 95 which the new alloys can be used for welding and brazing purposes and of the strong joints which it produces, they can be used to great advantage in the manufacture of electrical machinery, for example, in the soldering of transformer leads. Also, since little or no flux is required, they may be used with excellent results in operations in which resistance heating is employed. 100

## What I claim:

1. An alloy which consists of silver varying 105 from about 4% to about 36%, copper varying from about 55% to about 80%, tin varying from about 5% to about 15%, and phosphorous varying from about 2% to about 6%. 110

2. An alloy which consists of about 4% silver, about 78.1% copper, about 13.4% tin, and about 4.8% phosphorus.

3. An alloy which consists of silver varying from about 14% to about 16%, copper varying from about 69% to about 71%, tin varying from about 11% to 12%, and phosphorus varying from about 3.5% to about 5.5%.

4. An alloy which consists of silver varying from about 24% to about 36%, copper varying from about 55% to about 64%, tin varying from about 7% to about 11%, and phosphorus varying from about 2% to about 3.5%.

80

ROBERT H. LEACH.

10

85

15

90

20

95

25

100

30

105

35

110

40

115

45

120

50

125

55

130

60

135

65

140

70

145

75

150